

May 4, 1926.

1,583,545

H. FROOD ET AL

PRODUCTION OF PATTERNED INDIA RUBBER

Filed Oct. 16, 1924



Inventors  
H. Frood & W.R. Sydee  
By  
Marks & Clerk

## UNITED STATES PATENT OFFICE.

HERBERT FROOD AND WALTER RICHARD SYDEE, OF CHAPEL-EN-LE-FRITH,  
ENGLAND.

## PRODUCTION OF PATTERNED INDIA RUBBER.

Application filed October 16, 1924. Serial No. 744,060.

*To all whom it may concern:*

Be it known that we, HERBERT FROOD and WALTER RICHARD SYDEE, British subjects, both of Sovereign Mills, Chapel-en-le-Frith,

5 in the county of Derby, England, have invented certain new and useful Improvements Relating to the Production of Patterned India Rubber, of which the following is a specification.

10 This invention has for its object the ready and convenient production of pattern effects in rubber goods such as tiles, sheets, tubes and other articles.

Our invention comprises the production 15 of a patterned effect in indiarubber goods by consolidating into a mass of the desired size and shape, sections or portions of rubber of any desired colour and shape the said sections being coated with metal before 20 such consolidation and the said coating removed from the exposed faces or surfaces of the sections after said consolidation.

In one convenient application of our invention, unvulcanized rubber sheets of the 25 desired colour are cut up into small sections which may be of regular or irregular shapes. The mixed coloured sections are then dipped or immersed in a solution consisting of a mixture of rubber solution and 30 metallic powder, such as aluminium powder, whereby the various sections become coated with an aluminium or other metal coating. The mass is then consolidated into sheet, tile or other form by suitable presses or by 35 passing the same through a roller or mangle type of machine. The sheets or tiles are vulcanized and their faces finished by grinding or otherwise removing the surface of the same whereby the metal coating is taken 40 therefrom and the variegated coloured pattern is exposed, each coloured section having a border or vein like surround of the aluminium or other metal, whereby desirable ornamental effects are obtained.

45 It will of course be understood that we may, if desired, coat some of the rubber sections with a metallic powder and use other sections which are uncoated so as to vary the final pattern produced.

50 We may, in some cases, provide a sheet

or solid base piece or backing with a covering of the mixed coloured sections instead of making the whole of the sheet of the mixed coloured sections.

The accompanying drawing illustrates the 55 face of a circular slab of rubber made up from a consolidated mass of metal coated rubber sections of various shapes, and colours, the metal being removed from the face of the sections after such consolidation. 60 The reference letter *a* indicates coloured rubber sections and the letter *b* the metal border or veins surrounding the sections.

We claim:

1. The process of producing a mosaic effect in indiarubber goods, consisting in coating a number of pieces of rubber with metal, uniting said coated pieces to form a unit of the required size and shape, and subsequently removing the metal coating from the top 70 of said unit thereby exposing the rubber surface of the constituent pieces aforesaid and the upper edges of the portions of the said coating on the contiguous sides of said pieces. 75

2. The process of producing a mosaic effect in indiarubber goods, consisting in cutting rubber sheets of different colours into small sections, dipping said sections in a metallic powder solution thereby giving them a metallic coating, uniting said metal coated sections into one unit, and subsequently removing the metal coating from the top of said unit thereby exposing the rubber surface of the respective sections and the upper edges of the portions of the coating on the contiguous sides of said sections. 80

3. The process of producing a mosaic effect in indiarubber goods, consisting in cutting sheet rubber into small sections, dipping some of the said sections in a metallic powder solution thereby giving them a metallic coating, uniting said metal coated sections with a number of uncoated sections to form one unit, and subsequently removing the metal from the top of said coated sections leaving exposed the upper edges of the metal coating on the sides of the sections. 85

4. The process of producing a mosaic ef- 90

100

fect in indiarubber goods, consisting in cutting rubber sheets into small sections, dipping said sections in a metallic powder solution thereby giving them a metallic coating, uniting said metal coated sections into one unit, removing the metal coating from the top of said unit leaving exposed the up-

per edges of the metal coating on the sides of the sections and providing a rubber base on the under surface of said unit.

10 In testimony whereof we have signed our names to this specification.

HERBERT FROOD.

WALTER RICHARD SYDEE.